

Patented June 26, 1928.

1,674,694

# UNITED STATES PATENT OFFICE.

EDWIN R. MILLRING, OF NEW YORK, N. Y., ASSIGNOR TO AMERICAN MACHINE & FOUNDRY COMPANY, A CORPORATION OF NEW JERSEY.

## PROTECTIVE COMPOSITION FOR METAL-COATING BATHS.

No Drawing

Application filed January 9, 1925. Serial No. 1,353.

This invention relates to that method of covering metals with a metallic protective coat or envelope, in which the article of metal to be coated is, after being suitably 5 cleansed and fluxed, immersed in a bath of molten coating metal. In the coating of certain articles, such for instance as metal sheets, the sheets after being passed through the bath of coating metal, are passed between metal rolls which act to smooth out 10 the metal coating and wring off the excess of the coating metal, and in order to protect the surface of the coating bath from oxidation, it has been the practice to cover the 15 same with an oil bath which surrounds and submerges the rolls. Palm oil, tallow, rosin oil and other oils have been used for this purpose, but have not proved satisfactory, because, at the high temperatures required 20 for the application of certain coating metals and alloys, firing of the oil may take place, or the same may rapidly carbonize, polymerize, or oxidize, and lose its virtue in protecting the surface of the coating bath.

25 As a result of experiments and operations carried out under practical conditions I have discovered a protective liquid which is suitable for protecting the surface of the metal coating bath against oxidation, where coating metals are employed requiring relatively 30 high temperatures for their application, such for instance as lead coatings and coatings of alloys of lead containing 16% or less of tin, which protective liquid possesses 35 properties which will prevent its deterioration, as by firing, carbonizing, polymerizing, or oxidation, under the relatively high temperature conditions required, and which by surrounding the rolls between which the 40 coated sheets are passed, will maintain said rolls at the relatively high temperature necessary for their proper functioning under the conditions mentioned.

In its preferred form, this protective 45 liquid is an oleaginous material, specifically rape seed oil, and may be used alone as a protective covering for the metal bath or it may be used in admixture with another ingredient such as a petroleum product, to 50 form an oil mixture possessing the properties and characteristics above mentioned, and the invention consists of the improved composition of matter consisting of an oil mixture possessing the above described 55 characteristics.

The protective liquid possessing the above mentioned properties, is preferably an oleaginous liquid, and may consist of rape seed oil which possesses a sufficiently high fire point to prevent firing and also possesses properties which will prevent its deterioration under the working temperature of the coating metal, and this oil will act therefore to protect the surface of the coating bath against oxidation under the temperature 65 conditions described.

In the use of the protective liquid it is placed on the surface of the metal coating bath so as to surround the usual rolls between which the sheets pass after leaving 70 the bath, the liquid thus surrounding the rolls acting to maintain them at the requisite high degree of temperature necessary for the performance of their functions in smoothing down the coating metal and 75 wringing off the excess thereof.

Instead of rape seed oil alone, I may employ the same in admixture with another ingredient, such as "Insulatum A-A," a highly refined petroleum product having a 80 fire point and boiling point in excess of 350° C. and free from tar and from which the unsaturated hydrocarbons have been largely removed, and which has been purified preferably by vacuum distillation, these ingredients to be mixed in the proportions of 98% or thereabout of refined rape seed oil and 2% or thereabout of insulatum. It will be understood that the specific ingredients of this oil mixture may be changed and modified without departing from the limits of 85 the invention, the essential requirement being that the oil mixture will possess the characteristics and properties hereinbefore described. The rape seed oil or the above described oil mixture, according to which may be employed, will, by surrounding the rolls between which the sheets are entered after 90 their passage through the molten coating bath, maintain said rolls at the high degree 100 of temperature necessary for them to perform their functions as described, and in addition will enable the rolls to give a finish to the coated sheets, known as an "oil finish."

While in the foregoing description I have 105 set forth the use of the protective liquid in connection with a molten bath of lead employed to coat metal sheets, it will be understood that the invention is not limited to this particular use, but is applicable as 110

well for the protection against oxidation of the surface of coating baths of other metals; and may be employed in connection with other forms of apparatus, and for the coating of other forms of metal articles. For instance in the coating of wire with a metal coating, the rolls would be omitted and a layer of sand placed on the surface of the bath together with the protective liquid so that in the passage of the wire through the sand layer, the surplus coating metal would be removed and the metal properly distributed in smooth condition on the wire.

A small quantity, say 3 to 5% of palm oil may be added to the oil mixture to assist in the application of tin or metal to the rolls, when it is found desirable to do so.

Having thus described my invention, what I claim is:

1. A composition of matter for protecting the surface of molten metal coating baths against oxidation, which consists of a mixture of rape seed oil and a petroleum product possessing a fire point in excess of 350° C.

2. A composition of matter for protecting the surface of molten metal coating baths against oxidation, which consists of a mixture of rape seed oil and insulatum in proportions substantially as described.

3. A composition of matter for protecting the surface of molten metal coating baths against oxidation, which consists of a mixture of 98% of rape seed oil and 2% of insulatum.

In testimony whereof, I have affixed my signature hereto.

EDWIN R. MILLRING.